

1

2,933,453

## PROCESS FOR THE DECONTAMINATION OF MUSTARD GAS-CONTAMINATED CARBON FABRIC

Dana Burks, Jr., Walpole, Mass., assignor, by mesne assignments, to the United States of America as represented by the Secretary of War

No Drawing. Application May 9, 1946  
Serial No. 668,469

6 Claims. (Cl. 252—412)

This invention relates to the decontamination of protective fabrics which have been contaminated by vesicant agents. More particularly this invention pertains to a method of decontaminating carbon-containing protective fabric which has been exposed to mustard gas.

It is an object of this invention to devise a process, for the decontamination of protective clothing, which will effectively and economically remove contamination by vesicant gases but which will not weaken the fabric.

Further objects will appear hereinafter.

In order to protect personnel and materiel against the action of vesicant agents, various types of protective fabrics have been designed. A recent innovation in this field has been fabrics impregnated with or coated with activated carbon. When these fabrics have been exposed to the action of a vesicant, such as mustard gas ( $\text{ClCH}_2\text{CH}_2\text{SCH}_2\text{CH}_2\text{Cl}$ ), they become contaminated by adsorption of the gas and must be decontaminated before they can be handled by unprotected personnel and before they can be reused.

It has long been known that mustard gas can be rendered inactive as a vesicant by reaction with bleaching powder and therefore it was attempted to employ a dilute aqueous solution of sodium hypochlorite, such as that employed in commercial bleaching of textile fabrics, to decontaminate carbon-coated protective fabrics which had been exposed to mustard gas vapor.

A sample of carbon-coated fabric was therefore allowed to adsorb mustard vapor to the point of saturation and was then regenerated by immersion in an aqueous sodium hypochlorite (0.2 percent available chlorine) solution for 15 minutes at room temperature, rinsed with water, "antichlorized" with dilute sulfuric acid, again rinsed with water and finally dried. Although the material had been completely regenerated it was found after four successive contaminations and decontaminations that the carbon-coated fabric had suffered a material decrease in tensile strength, a condition which was occasioned by the repeated applications of sodium hypochlorite and dilute acid followed by drying.

I have discovered that the disadvantage exhibited in the use of sodium hypochlorite can be overcome when a dilute, aqueous, neutral, solution of hydrogen peroxide, either *per se*, or produced *in situ*, is used as the decontaminating agent. Vesicants are removed effectively without decreasing the tensile strength of the material. The use of hydrogen peroxide in my preferred embodiment has the additional advantage over bleach solutions in that no rinsing following decontamination and prior to drying.

While I have found, because of the latter advantage, and in the interest of economy, that hydrogen peroxide is to be preferred, other peroxides are operative and the hydrogen peroxide can be generated *in situ* to produce

2

effective decontamination. My invention therefore can be performed by any composition which will produce a neutral solution of hydrogen peroxide in water.

A specific example of the preferred method performing my invention is as follows:

### EXAMPLE 1

Samples of carbon-coated fabric were contaminated with mustard gas (HS) by being exposed to mustard gas vapor to the point of saturation. The samples were then placed in a 2.0 percent aqueous solution of neutral hydrogen peroxide at room temperature. The samples were then dried for 5 minutes at 250 deg. F. without rinsing. The protective value of the decontaminated fabric after treatment was not significantly different from its initial value, as indicated by the data set forth in Table I below. After nine contamination and decontamination cycles, performed as above, the protective value of the fabric was still not significantly different from its initial value as indicated by the data shown in the table below, and at the end of the 9th regeneration no decrease in the tensile strength of the fabric could be determined.

Table I.—Regeneration of carbon coated protective fabric, following saturation with HS vapor, by means of neutral hydrogen peroxide

Regeneration Procedure:

(a) 21 samples of contaminated fabric (total weight 8.4 grams) immersed in 2 liters of 2 per cent hydrogen peroxide.

(b) Decontaminated samples dried 5 minutes at 250° F. with no rinsing.

(c) Protective value determined by "Spotted Dick" procedure.

The "Spotted Dick" test used in testing my fabrics is conducted as follows: A single drop of liquid mustard is placed in the center of a cellophane disk (.0015" thick) which in turn is located at the bottom of a circular depression (.75" diameter, 0.125" deep) in a solid brass plate. The test fabric is placed over the depression. On the test fabric is placed in successive order (1) an alkaline filter paper, and (2) an indicator paper, dyed with Congo Red and subsequently spotted, through a perforated cellophane sheet, with a tetrachlorethane solution of 1,3,4,6-tetrachloro 7,8-diphenylglycoluril (saturated at 25° C.). The whole assembly is then held in place by a heavy glass plate. The period required for mustard vapor to penetrate the fabric and to cause the indicator paper to change in color, is defined as the Penetration Time or the Protective Time.

| Sample Number           | Number of Regeneration Cycles |     |    |
|-------------------------|-------------------------------|-----|----|
|                         | 0                             | 1   | 9  |
| Protective Time—minutes |                               |     |    |
| 1                       | 67                            | 79  | 63 |
| 2                       | 78                            | 88  | 53 |
| 3                       | 55                            | 62  | 48 |
| 4                       | 60                            | 77  | 53 |
| 5                       | 77                            | 63  | 79 |
| 6                       | 66                            | 62  | 79 |
| 7                       | 61                            | 55  | 52 |
| 8                       | 84                            | 92  | 65 |
| 9                       | 77                            | 80  | 78 |
| 10                      | 48                            | 90  | 83 |
| 11                      | 63                            | 79  | 69 |
| 12                      | 58                            | 70  | 66 |
| 13                      | 65                            | 77  | 45 |
| 14                      | 63                            | 50  | 63 |
| 15                      | 87                            | 85  | 53 |
| 16                      | 52                            | 99  | 42 |
| 17                      | 59                            | 76  | 77 |
| 18                      | 72                            | 99  | 47 |
| 19                      | 73                            | 52  | 63 |
| 20                      | 73                            | 46  | 50 |
| 21                      | 83                            | 102 | 41 |
| Mean                    | 68                            | 75  | 60 |

In order to determine the optimum regeneration time, tests were run, in which the fabric samples were subjected to the action of hydrogen peroxide for 5, 10, 30, 60, and 120 minutes. The results of these tests are given in Table II below and the data indicates that complete regeneration is effected in a relatively short time,

Table II.—Regeneration with hydrogen peroxide effect of time

| Regeneration Time—minutes..... | "Spotted Dick" Protective Value—minutes |      |      |      |      |
|--------------------------------|-----------------------------------------|------|------|------|------|
|                                | 5                                       | 10   | 30   | 60   | 120  |
|                                | 63                                      | 77   | 62   | 88   | 79   |
|                                | 62                                      | 55   | 62   | 80   | 90   |
|                                | 85                                      | 50   | 77   | 70   | 79   |
|                                | 46                                      | 52   | 79   | 76   | 99   |
| Mean.....                      | 64.0                                    | 58.5 | 77.5 | 78.5 | 86.8 |

Although the use of hydrogen peroxide per se has the advantage that rinsing is not required, from a standpoint of application in the field, a definite limitation is placed on its use, since it would be impractical to add concentrated hydrogen peroxide to a combat kit. Therefore, I have determined that dry mixtures which produce hydrogen peroxide in water solution can be employed. Many such compositions are known. I have found that the following composition is especially effective:

A 50:50 mixture of sodium perborate monohydrate and sodium dihydrogen phosphate monohydrate (Kharasch Mixture) which yields a neutral solution of hydrogen peroxide when dissolved in water, and is capable of effectively decontaminating fabrics in a manner comparable to dilute hydrogen peroxide per se, for example.

#### EXAMPLE 2

Samples of carbon-coated protective fabric contaminated with mustard gas by saturation with mustard vapor were placed in a solution prepared by dissolving 12.6 grams of a 50:50 mixture of sodium perborate monohydrate and sodium dihydrogen phosphate monohydrate in a 100 cc. of water (equivalent to a 2% solution of  $H_2O_2$ ). Following decontamination, the residual products of the sodium perborate-sodium dihydrogen phosphate reaction were removed from the fabric by repeated rinsing with water and the decontaminated fabric was dried. This fabric then exhibited protective properties comparable to that of uncontaminated controls as indicated by the data presented in Table III below.

Table III.—Regeneration with hydrogen peroxide neutral hydrogen peroxide vs. solution prepared from Kharasch's 50:50 mixture of sodium perborate and sodium dihydrogen phosphate

[<sup>40</sup> "Spotted Dick" protective time—  
minutes.]

The nature of this invention has been broadly outlined above, the preferred embodiments have been described and it will be apparent that certain modifications and additional formulations will suggest themselves to those skilled in the art. Accordingly, it is intended that the foregoing description shall be interpreted as illustrative only and not in a limiting sense.

I claim:

1. A process for decontaminating carbon-coated protective fabric which has been exposed to the action of mustard gas, comprising treating said fabric with a solution of neutral hydrogen peroxide produced in situ by action of water with a dry mixture of sodium perborate monohydrate and sodium dihydrogen phosphate monohydrate producing neutral hydrogen peroxide in water.
- 10 2. A process for decontaminating carbon-coated protective fabric which has been exposed to the action of mustard gas, comprising treating said fabric with a dilute solution of neutral hydrogen peroxide.
- 15 3. A process for decontaminating carbon-coated protective fabric which has been exposed to the action of mustard gas, comprising treating said fabric with an aqueous of sodium perborate monohydrate and sodium dihydrogen phosphate monohydrate.
- 20 4. A process for decontaminating carbon-coated protective fabric which has been exposed to the action of mustard gas, comprising treating said fabric with a neutral 2 percent aqueous solution of hydrogen peroxide.
- 25 5. A process for decontaminating carbon-coated protective fabric which has been exposed to the action of mustard gas, comprising treating said fabric with a neutral 2 percent aqueous solution of hydrogen peroxide at room temperature.
- 30 6. A process for decontaminating carbon-coated protective fabric which has been exposed to the action of mustard gas, comprising treating said fabric for at least 5 minutes with a neutral 2 percent aqueous solution of hydrogen peroxide.

#### References Cited in the file of this patent

#### UNITED STATES PATENTS

|           |            |       |                |
|-----------|------------|-------|----------------|
| 916,692   | Foregger   | ----- | Mar. 30, 1909  |
| 1,160,563 | Barrington | ----- | Nov. 16, 1915  |
| 1,353,654 | Harrison   | ----- | Sept. 21, 1920 |
| 2,054,885 | Schroter   | ----- | Sept. 22, 1936 |
| 2,394,887 | Berl       | ----- | Feb. 12, 1946  |
| 2,396,923 | Mendelsohn | ----- | Mar. 19, 1946  |
| 2,465,228 | Hein       | ----- | Mar. 22, 1949  |

#### FOREIGN PATENTS

|         |               |       |              |
|---------|---------------|-------|--------------|
| 496,752 | Great Britain | ----- | Dec. 1, 1938 |
|---------|---------------|-------|--------------|

| Uncon-taminated Controls | Decontaminated Fabrics |                   |
|--------------------------|------------------------|-------------------|
|                          | Hydrogen Peroxide      | Kharasch Solution |
| 48                       | 44                     | 42                |
| 34                       | 51                     | 46                |
| 44                       | 57                     | 48                |
| 33                       | 45                     | 45                |
| 33                       | 56                     | 41                |
| 39                       | 45                     | 44                |
| Mean—38.5                | 46.9                   | 44.3              |

UNITED STATES PATENT OFFICE  
CERTIFICATE OF CORRECTION

Patent No. 2,933,453

April 19, 1960

Dana Burks, Jr.

It is hereby certified that error appears in the printed specification of the above numbered patent requiring correction and that the said Letters Patent should read as corrected below.

Column 1, line 63, after "rinsing" insert -- is required --;  
column 4, line 23, after "aqueous" insert -- solution --.

Signed and sealed this 13th day of September 1960.

(SEAL)

Attest:

KARL H. AXLINE  
Attesting Officer

ROBERT C. WATSON  
Commissioner of Patents